

# UNITED STATES PATENT OFFICE.

WILLIAM HENRY PERKIN, JR., OF MANCHESTER, ENGLAND, ASSIGNOR OF ONE-HALF TO WHIPP BROTHERS & TOD, LIMITED, OF MANCHESTER, ENGLAND.

## PROCESS OF FIREPROOFING TEXTILE MATERIALS.

No. 856,906.

Specification of Letters Patent.

Patented June 11, 1907.

Application filed May 10, 1902. Serial No. 106,837.

*To all whom it may concern:*

Be it known that I, WILLIAM HENRY PERKIN, Jr., Ph. D. F. R. S., a subject of the King of Great Britain and Ireland, residing at 5 Owen's College, in the city of Manchester, in the county of Lancaster, England, professor of organic chemistry, have invented certain new and useful Improvements in the Treatment of Raw Cotton and Flax and Cotton and Linen Goods to Reduce the Inflammability Thereof; and I do hereby declare the following to be a full, clear, and exact description of the invention, such as will enable others skilled in the art to which it appertains to 15 make and use the same.

This invention relates to the treatment of raw cotton and flax and cotton and linen goods generally, (and especially the fluffy cotton goods known as flannelette) for rendering them less inflammable than hitherto by fixing an insoluble compound in the fibers of the material, so that they can be repeatedly washed and still retain their resistance to ignition.

25 The object of this invention is to effect improvements and modifications on the process, for which I have obtained Letters Patent No 844,042, Feb. 12, 1907.

The following are examples of ways in 30 which this invention may be performed, as applied, for example, to flannelette of medium quality, but the invention is not limited to these examples (the parts are by volume);

35 Example I. The goods are treated with a stannate of soda solution of 1.100 specific gravity and are then dried and afterward treated with a bath made up of equal parts of tungstate of soda solution of 1.300 specific gravity, and of ammonium chlorid solution of

1.050 specific gravity and one part of ammonia solution of .880 specific gravity. The goods are then dried, or dried and steamed.

Example II. The goods are treated with a stannate of soda solution of 1.100 specific gravity and are then dried and afterward 45 treated with a bath made up of seven parts of tungstate of soda solution of 1.300 specific gravity, three parts of acetic acid of 1.050 specific gravity and four parts of ammonium chlorid solution of 1.050 specific gravity. The 50 goods are then dried, or dried and steamed.

It is preferred in treating woven goods and the like, as aforesaid, to remove "sizing" before the treatment, but this is not essential.

I claim as my invention:

1. The herein described process of rendering textile materials less inflammable, said process consisting in fixing an insoluble compound in the fibers of the material by subjecting the material to the action of a soluble 60 stannate, then drying and then subjecting the material to the action of a bath containing a salt of ammonium, substantially as described.

2. The herein described process of rendering textile materials less inflammable, said process consisting in fixing an insoluble compound in the fibers of the material by subjecting the material to the action of a soluble stannate, then drying and then subjecting the 7c material to the action of a bath containing a soluble tungstate and a salt of ammonium.

In testimony whereof I affix my signature in the presence of two witnesses.

WILLIAM HENRY PERKIN, JUNIOR.

Witnesses:

W. GERALD REYNOLDS,  
PERCY READ GOLDRING.